

## UNITED STATES PATENT OFFICE

2,680,890

## REFRACTORY INVESTMENT AND MOLD

Thomas E. Moore and Claude H. Watts, Toledo,  
Ohio, assignors to The Ransom and Randolph  
Company, Toledo, Ohio, a corporation of Ohio

No Drawing. Application March 2, 1950,  
Serial No. 147,328

6 Claims. (Cl. 22—113.1)

1

This invention relates to refractory investments particularly useful in the casting of metals melting over 2300° F. particularly dental castings of the chrome-cobalt type, to investment compositions useful in producing such investments, to molds made with such investment compositions, to methods of making such compositions, investments, molds, and castings, and their utilization.

The invention is particularly concerned with such compositions, articles, and methods desirably used in the manufacture of smooth precision castings of intricate shape by the so called lost-wax method. This type of method may well be illustrated by the steps used in making dental castings generally as follows:

1. An impression is taken of the mouth with an elastic type impression material.

2. A master model is made by pouring a mix of dental stone (calcium sulfate hemi-hydrate composition) into the impression.

3. An impression is taken of the master model, using a duplicating material which is usually a gelatin base. (Korogel or hydrocolloid materials are sometimes used, but gelatin base impressions have been most satisfactory.)

4. A mix of the investment material is made and vibrated into the impression.

5. After the investment has set, it is removed from the impression and wax is flowed and adapted onto the model and around the teeth to form the clasps and the remainder of the dental appliance that it is desired to reproduce as a metal casting.

6. The "waxed up" model with adequate sprues attached is then placed in a flask which is filled with an outer investment.

7. After the outer investment has set, the flask is fired to 1400° F. or higher to remove all traces of wax and moisture and to expand the mold.

8. Molten metal is cast into the hot investment mold, usually with a centrifugal casting machine.

9. The casting is removed from the investment material.

In carrying out such methods, various types of investment compositions have been used. Thus an investment material consisting essentially of silica flour and bonded by an acidified organic silicate such as ethyl silicate is well known in the art. Further it is known to use investment materials that are bonded by mixing with dilute acids. These compositions have presented certain difficulties however which have been more or less objectionable in their utilization. In the case of the ethyl silicate bonded investment, it

2

is necessary to tamp the investment for several hours after pouring up the model in order to compact the mold so that it will be hard and dense enough for practical use. The bond is also very slow to set up for the model to be hard enough to work on. The tamping operation is objectionable because it is awkward, clumsy, and time consuming—and in many instances is likely to be deleterious to the accuracy of the finished casting. Investments mixed with dilute acids have been unsatisfactory because they do not attain sufficient strength on setting at room temperature to make a good model. Also the surface of the investment next to the model does not separate cleanly, but leaves a rough surface which is not an accurate reproduction of the impression taken in the mouth.

Other difficulties have been experienced with other types of investment materials. Thus calcium sulfate bonded investment decomposes at the temperature of the high melting metals to which particular reference has been made above.

Among the objects of the present invention is included refractory investment material for casting partial and full dentures of high fusing alloys.

Other objects include the utilization of two different types of investment materials in the production of a mold one composition particularly being used for the model investment and the other for the outer investment as more particularly further described below, the two investments varying in properties to give complete control of the operation and elimination of difficulties of the prior art.

Other objects of the invention include a model investment that will set rapidly and attain sufficient surface hardness and strength without tamping so that it may be removed from the duplicating material in approximately one hour or other relatively short space of time without breaking the teeth or other parts of the model, producing a clean sharp cast.

Still other objects include investment of sufficient hardness to permit handling and manipulation during the waxing operation without scratching or other impairment of the surface by waxing instruments used or by the fingers of the manipulator.

Still further objects include investment materials of sufficient setting and thermal expansion to compensate for the casting shrinkage of the metal.

Still further objects and advantages of the

present invention will appear from the more detailed description set forth below, it being understood that such more detailed description is given by way of illustration and explanation only, and not by way of limitation, since various changes therein may be made by those skilled in the art without departing from the scope and spirit of the present invention.

In the present invention one of the particularly emphasized features is the discovery that it has been found desirable to use two separate and distinct investment materials, one for the model investment and the other as an outer investment, each investment having controlled physical properties, and the investment compositions being particularly compounded for use with each other, in the production of refractory molds which solve many of the difficulties in the art. The utilization of two different types of investments namely a model investment and an outer investment enables the properties of each of the investments to be controlled to give the most desirable properties for the particular purpose or function for which each investment is adapted and yet enabling the investments to be formulated for use with each other in order to secure the objects sought. While particular types of investment compositions are herein set forth as most particularly valuable for present purposes, there are certain general considerations and relations between the two types of investments that are particularly important in the casting of the high fusion metals as set forth above for these purposes. Thus it has been found that the outer investment need not be as hard as the model investment and therefore the outer investment may exhibit a lower compression strength than the model investment. It has also been found that the setting expansion of the outer investment should not be more than .2% and that the thermal expansion of the outer investment should not be more than the thermal expansion of the model investment. These expansion limitations are necessary to prevent the outer investment from expanding away from the model, which would obviously result in undesirable flash on the finished casting. By the production of two different types of investment materials insofar as such setting and expansion properties are concerned, they may be controlled to give the most desirable set of properties in the particular investment considering the purpose which it serves and the manner in which it is used.

The investment compositions employed in the production of the model investment and of the outer investment may be substantially different in character as long as they possess the essential characteristics in their relation one to the other as pointed out above and exhibit otherwise properties enabling their utilization in the casting of metals which melt above 2300° F. But desirably both the model and outer investment compositions may generally be made of the same types of materials within the limits and with modifications as set forth below to adjust the properties thereof for the purposes set forth above. The most desirable types of materials that may be utilized as the basis for the investment compositions for both the model and outer investments may be produced from compositions which contain a major amount of a refractory material and a minor amount of binding and setting agents such as water soluble acid phosphate salts and basic material utilized therewith. The

refractory material employed particularly for dental purposes will generally be silica particularly compositions made up of graded silicas of different mesh using for example a balanced composition of silica running from about 30 mesh, through 50 mesh, 100 mesh and 200 mesh for example to give the desired graded composition for such purpose. Other refractory materials may be employed, many such materials being available in the art. The silica may be in any of its various forms such as quartz, tridymite, cristobalite, and also hydrated forms such as silicic acid, tripoli, diatomaceous earth, etc. Silica is the most desirable refractory material because it is inexpensive and because it forms a satisfactory high temperature bond with the phosphate. Other oxides of the silicon group may be used in place of silicon dioxide either in whole or in part such as the oxides of titanium, zirconium, and thorium; and other refractory materials such as nonplastic refractory clays, fire clay, kaolinite, sillimanite, andalusite, mullite, silicon carbide, zirconium silicate, titanium silicate, the spinels, refractory aluminum oxide, etc., may be used either in whole or to replace at least a part of the silica if desired, or various combinations of these different refractory materials may be utilized, particularly for the outer investment. The model investment should exhibit a high thermal expansion, so that the refractory used therein should be selected with this in view; and accordingly may desirably consist chiefly of silica or cristobalite. Additions of other silicates or refractory metal oxides should be held to a minimum, or used in the smallest per cent possible to give the desired property. For example the addition of zirconium silicate to the model investment actually reduces the thermal expansion, but the surface hardness and strength are considerably increased. The invention however will be particularly illustrated by the use of silica.

A water soluble acid phosphate salt is desirably used in the composition particularly balanced mixtures of such acid phosphates. Compounds producing  $P_2O_5$  at elevated temperatures may comprise acid salts of ortho, meta, and pyrophosphoric acid with lithium, magnesium, calcium, ammonium, strontium, barium, copper, zinc, cadmium, etc. Also, besides ammonium phosphate, there may be used the organic amino compounds such as primary, secondary, and tertiary methyl, ethyl and n-propyl amine phosphates. However, any large quantity of ammonia or other gas driven off during heating is undesirable. Of these various alkali metal and alkaline earth metal salts, etc., mono ammonium phosphate and mono magnesium phosphate are preferred because they are available in commercial quantities.

The basic material should be carefully chosen for reaction with the phosphate to give the composition the desired setting and other properties. Basic materials including the oxides and hydroxides of calcium, strontium, zinc, cadmium, copper, lithium, and barium, give investments which are too soft for the purposes of this invention. Fused magnesium oxide is therefore desirably used.

Considerations governing the utilization of these components of the investment compositions and other features involved in the invention can best be left until after a consideration of formulations that may be desirably employed and illustrate important features of the present invention.

To illustrate the composition used for the model investment the following is given:

I. FORMULA FOR MODEL INVESTMENT

7% fused magnesium oxide—325 mesh  
 3% powdered mono magnesium phosphate  
 9% powdered mono ammonium phosphate  
 20% milled zirconium silicate—325 mesh  
 20% silica—50 mesh  
 10% silica—30 mesh  
 31% silica—200 mesh

This investment composition has a refractory grain size gradation such that a minimum of liquid is required to make a putty-like mix that will flow under gentle vibration.

Representative formulas for the model investment illustrating limits for the fused magnesium oxide which desirably may be from 5% to 10% and limits for the soluble acid phosphate salts which desirably may be from 10% to 17.5% are as follows:

No. 1 (Low limit)

5% fused MgO—325 mesh  
 4%  $Mg(H_2PO_4)_2$   
 6%  $NH_4H_2PO_4$   
 20% milled zirconium silicate—325 mesh  
 20% 50 mesh silica  
 10% 30 mesh silica  
 35% 200 mesh silica

W/I (water to investment composition) =  
 10/100 liquid 18% silica sol

No. 2 (High limit)

10.0% fused MgO—325 mesh  
 4.5%  $Mg(H_2PO_4)_2$   
 13.0%  $NH_4H_2PO_4$   
 20.0% milled zirconium silicate—325 mesh  
 20.0% 50 mesh silica  
 10.0% 30 mesh silica  
 22.5% 200 mesh silica

W/I=10/100 liquid 18% silica sol

Formula No. 1 may be used with some success, but the strength is somewhat lower than that required for a good model, and the teeth are apt to break off on removing the model from the duplicating material. Also the model tends to develop small cracks on setting at room temperature after removing from the duplicating material. Formula No. 2 is very satisfactory and although higher percentages of fused magnesium oxide and phosphate salts could be used with some success, the thermal expansion of such formulas would not be sufficiently high and the resulting castings would be under size.

It is not absolutely necessary to use zirconium silicate (zirconite, etc.) in the model investment. A satisfactory and workable formula can be compounded using silica only, in varying mesh sizes, for the refractory filler as taught herein. However, the preferred formula does contain 20% zirconium silicate because the surface hardness is increased, and from 5% to 25% of zirconium silicate may be used, desirably for this purpose. Other refractory materials among those mentioned above may be used to replace zirconium silicate in whole or in part with similar beneficial results.

It has been found that in lieu of using water for addition to such composition to produce the investment material, superior results are obtained by the utilization of silica sol such as that manufactured by National Aluminate Corporation or by Du Pont under the name of "Ludox." Such silica sols are represented by those set forth in

U. S. Patent No. 2,244,325. Silica sol used in this way has been found to have a very important efficacious effect in the nature of the investment produced particularly from compositions of the character set forth above and modifications thereof as hereinafter taught. The use of silica sol in this way particularly within restricted concentrations will increase the setting expansion and also increase the hardness of the model, which makes for a smoother, harder surface both of which are desirable properties. Silica sol is available commercially either in 18% or 30% concentration, and by dilution any concentration of silica sol up to 30% may be used with corresponding variations in expansion properties, hardness, and compression strength. In some applications a silica sol concentration of as low as 2% concentration has shown a noticeable increase in setting expansion and hardness. While the 30% silica sol concentration may be used in some applications, generally the hardness and density of the investment when using such 30% silica sol concentration is increased to the point where the investment is not sufficiently permeable to allow the metal to cast out during the casting operation and gas pockets may be found in heavy sections. Consequently in general the concentration used particularly in connection with the casting of metals in accordance with the present invention is less than 30% for example between 2 and 21% and particularly important effects are obtained with concentrations of between 10 to 21% and specifically by the use of a solution of silica sol of 18% concentration. Specifications for 30% and 18% silica sol are as follows:

|    |                                    | 30%     | 18%  |
|----|------------------------------------|---------|------|
| 40 | Silica as $SiO_2$ .....            | percent |      |
|    | Soda as $Na_2O$ maximum.....       | do      | 0.3  |
|    | Sulfate as $Na_2SO_4$ maximum..... | do      | 0.09 |
|    | pH (approximately).....            | 10      | 10   |
|    | Pounds per Gallon.....             | 10      | 9.3  |

To illustrate the ratios in which it is used, the formulation as given above (No. 1) for the model investment when mixed with 18% silica sol in the proportions of 10 c. c. of 18% silica sol to 100 grams of model investment, gives the following physical properties in the investment:

50 Initial setting time  
 (Vicat needle) ..... 6 mins.  
 Compression strength, 2 hrs. 2000 lbs. per sq. in.  
 Setting expansion—Max.  
 3 hrs. ..... .85%  
 55 Thermal expansion—Max.  
 1400° F. ..... .60%

The following table shows setting expansion of Investment, Formula No. 1 for varying per cents of  $SiO_2$  sol in mixing water, using liquid-investment ratio of 10 c. c. to 100 grams:

| 65              | Percent $SiO_2$ Sol in Liquid | Percent Set. Expansion |
|-----------------|-------------------------------|------------------------|
| No $SiO_2$ Sol  |                               | 0.23                   |
| 6% $SiO_2$ Sol  |                               | 0.24                   |
| 10% $SiO_2$ Sol |                               | 0.43                   |
| 15% $SiO_2$ Sol |                               | 0.57                   |
| 18% $SiO_2$ Sol |                               | 0.80                   |
| 21% $SiO_2$ Sol |                               | 0.62                   |

This chart shows an increase in setting expansion as the per cent  $SiO_2$  sol in the mixing liquid is increased up to a maximum for 18%  $SiO_2$ . A further increase in per cent  $SiO_2$  to 21% gave a lower setting expansion than the 18% concen-

tration. Different investment compositions will give varying setting expansions for the same concentration of silica sol.

For example, the following formula, when mixed in the proportion of 10 c. c. liquid to 100 grams investment, gave setting expansions shown below.

| Percent SiO <sub>2</sub><br>Sol. | Percent Set.<br>Exp. |
|----------------------------------|----------------------|
| 18                               | 1.07                 |
| 21                               | 1.17                 |

Formula 3

8.5% fused MgO—325 mesh  
4.5% Mg(H<sub>2</sub>PO<sub>4</sub>)<sub>2</sub>  
13.0% NH<sub>4</sub>H<sub>2</sub>PO<sub>4</sub>  
20.0% Zirconite—325 mesh  
20.0% 50 mesh silica  
10.0% 30 mesh silica  
24.0% 200 mesh silica

A remarkable increase in setting expansion has been noted for some investment compositions when as small an amount as 2% SiO<sub>2</sub> sol was present in the mixing liquid.

It is preferred as shown in the formulations set forth herein, in the production of satisfactory investment to have primary binding ingredients other than silica sol present to give workable material, the additions of silica sol being used to enhance the end result due to increased hardness and increased setting expansion giving smoother surface on the cast metal and better fit.

These considerations will show the excellent results obtained by the use of the silica sol with investment compositions particularly those of the character herein set forth. However such silica sol may be desirably used as the bonding material with various types of setting refractory investments whether of the type set forth herein or of other types. But the use with the particular types of investment materials produced from refractory materials, water soluble acid phosphates salts, and basic materials of the character hereinabove set forth, gives unique results in the industry.

To illustrate considerations in connection with the outer investment, the following composition is illustrative:

## II. FORMULA FOR OUTER INVESTMENT

8% fused magnesium oxide—325 mesh  
9% powdered mono ammonium phosphate  
5.5% powdered mono magnesium phosphate  
27% 50 mesh silica  
25% 100 mesh silica  
25.5% 200 mesh silica

This formulation when mixed with water in the proportions for example of 18 c. c. water to 100 grams of outer investment gives the following physical properties in the resulting investment:

Initial setting time (Vicat needle) 10 mins.  
Compression strength, 2 hrs. 1140 lbs. per sq. in.  
Setting expansion, maximum .04%  
Thermal expansion .30%

Representative formulas for the outer investment illustrating limits for the fused magnesium oxide which desirably may be from 4% to 10%.

and limits for the soluble acid phosphate salts which desirably may be from 7.25% to 18.2% are as follows:

### No. 4 (Low limit)

4.00% fused MgO—325 mesh  
2.75% Mg(H<sub>2</sub>PO<sub>4</sub>)<sub>2</sub>  
4.50% NH<sub>4</sub>H<sub>2</sub>PO<sub>4</sub>  
27.00% 50 mesh silica  
25.00% 100 mesh silica  
36.75% 200 mesh silica  
W/I=18/100 using water for mixing

### No. 5 (High limit)

10.0% fused MgO—325 mesh  
6.9% Mg(H<sub>2</sub>PO<sub>4</sub>)<sub>2</sub>  
11.3% NH<sub>4</sub>H<sub>2</sub>PO<sub>4</sub>  
27.0% 50 mesh silica  
25.0% 100 mesh silica  
19.8% 200 mesh silica  
W/I=18/100 using water for mixing

As explained above it is important to produce an outer investment showing a controlled setting expansion of not over .2%. It has been found possible to make an investment that will meet this setting expansion requirement by control of the balance between the alkali used and the soluble acid phosphate salts in compositions of the character particularly illustrated above and more specifically when fused magnesium oxide is employed as the alkaline material for which it is most desirably suited as against the other alkaline materials although the latter may be employed. An important consideration in producing such low setting expansion with compositions of this type is in the utilization of sufficient fused magnesium oxide for example so that there will be an excess of such oxide after all of the soluble acid phosphate salts have been neutralized. In the particular formulation as given above calculation will show that for 100 grams of material of the formulation there given for the outer investment, 6.76 grams of MgO are required for neutralization of the soluble acid phosphate salts present whereas 8 grams are present in the formulation so that there is an excess of 1.24 grams of magnesium oxide per 100 grams of the stated additive investment composition above that necessary for neutralization of all of the soluble acid phosphate salts present. The excess magnesium oxide which may be present for this purpose beyond that necessary to neutralize all of the soluble acid phosphate salts in such compositions may be varied but should not be excessive. For example satisfactory results are obtained if the amount of magnesium oxide in excess of that necessary to neutralize the phosphate salts present is from 1 to 3%.

It is not necessary to use zirconium silicate in the outer investment, but it can be used if desired, and offers one way to control the thermal expansion so that it would not be greater than that of the model investment. However, the added strength is not required, and the higher cost more or less discourages its use here.

With regard to particle size of the fused magnesia for use both in the model investment and in the outer investment, both sizes may desirably be minus 325 mesh, i. e. 100% through 325 mesh. Differences between the particle size in the different investments require a determination of particle size below .5 micron, in connection with which it may be noted that there is no generally

accepted method for accurately measuring particles of this size. As exemplary of particle size desirably used for the specific purposes herein emphasized, the particle size of the fused magnesia will desirably be below 10 microns. While other size particles may be employed in investment materials the particle sizes herein set forth, give unique results for the particular purposes described.

Differences in particle size of the fused magnesium oxide have been pointed out above as desirable to obtain the best results. Another difference preferably used is in the amount of water employed in making the mix. A ratio of 10 c. c. liquid to 100 grams of model investment gives a very thick mix, which in turn makes for a harder and a stronger model. The consistency is such that it will flow under slight vibration. A ratio of 18 c. c. water to 100 grams of outer investment gives a fairly thin mix that can be painted onto the waxed up model. The consistency is such that the investment can be poured without vibration. It should be noted that the stated ratios of water or silica sol, as the case may be, to investment composition, as given above, are optimum ratios. These ratios may vary in each investment material but those set forth give the best effects.

The ratios and proportions of the components of the investment materials as exemplified above, and generally in the ranges of from 4-10% of magnesia, from about 7-7.25% to 18-18.2%, balance refractory (all ratios by weight), should in all cases be balanced to give the desired properties in the finished product. Ordinarily the fused magnesium oxide and soluble acid phosphate salts should be in the ratio of about 4:7 specifically 4:7.25, for the best results, but variation in this ratio within limits as herein taught may be used where the optimum effects are not essential. In addition, much better results are obtained by using a balanced formula of mixture of acid phosphate salts than by the use of a single acid salt in the composition. For example mono magnesium phosphate alone or mono ammonium phosphate alone is not as satisfactory as a mixture of them in balanced proportions. Generally speaking, in such a mixture, the mono magnesium phosphate should comprise from 25% to 40% by weight of the soluble acid phosphate salts present.

As overall values, the outer investment composition should contain by weight a major amount, not less than 70% of refractory material and a minor amount, not more than 20% of water-soluble acid phosphate salt, the balance being the magnesium oxide. More specifically there will be from 89% to 71.8% of refractory material, from about 7% to 18.2% of water soluble acid phosphate salt and from 4 to 10% of magnesium oxide.

For the model investment composition the preferred ratios are from about 72.5% to 85% of refractory material, from about 17.5% to 10% of water soluble acid phosphate salt, and from about 10% to 5% of fused magnesium oxide. And as stated with the model investment composition a silica sol of from 2 to 30% concentration by weight is desirably used as the liquid for addition to the composition.

The utilization of silica sol as set forth herein in phosphate type investments gives important results as pointed out above. Silica sol may also be used with other phosphate type investments particularly where the refractory material is

bonded by the use of acid phosphates in combination with basic material. Thus silica sol may be used with any of the investment compositions as set forth in Patent No. 2,479,504. It may be used in those combinations of the patent by employing as liquid for admixture with the solids, a silica sol of from 2 to 30% concentration by weight preferably using from 10 to 21% as also set forth above. In this way there is obtained increased hardness and increased setting expansion, giving smoother surface on cast metal and better fit.

Having thus set forth our invention, we claim:

1. In combination, a refractory mold for use in casting metals melting at over 2300° F. comprising a model investment, a wax pattern one face of which is in contact with said model investment, and an outer investment in contact with another face of said pattern, the outer investment differing in composition from the model investment and having a lower compression strength than the model investment, a thermal expansion not greater than that of the model investment, and a setting expansion of not more than .2% the model investment consisting essentially by weight of from 89% to 71.9% of a refractory material, from 7% to 18.2% of a water-soluble acid phosphate salt and from 4% to 10% of magnesium oxide, in which 5% to 25% by weight of the refractory material is zirconium silicate, and the outer investment consisting essentially by weight of from 89% to 71.8% of a refractory material, from 7% to 18.2% of a water-soluble acid phosphate salt and from 4% to 10% of magnesium oxide, the outer investment being substantially free from zirconium silicate.

2. A combination as set forth in claim 1, in which the model investment is bonded with silica sol of from 2 to 30% concentration in the ratio of 100 gms. of model investment composition to 10 c. c. to 18 c. c. silica sol.

3. In combination, a refractory mold for use in casting metals melting at over 2300° F. comprising a model investment and an outer investment, the investment compositions being different but each consisting essentially of by weight from 89% to 71.8% of a refractory material, from 7% to 18.2% of a water soluble acid phosphate salt, and from 4% to 10% of magnesium oxide, the ratio of salt to oxide being about 7:4 in which 5% to 25% by weight of the refractory material of the model investment is zirconium silicate, the outer investment being substantially free from zirconium silicate.

4. A model investment for use in casting metals melting at over 2300° F. comprising by weight from 72.5% to 85% of a refractory material, from 17.5% to 10% of a water soluble acid phosphate salt, and from 10% to 5% of fused magnesium oxide, and in which from 5% to 25% by weight of the refractory material is zirconium silicate, bonded with silica sol in the ratio of 100 gms. investment composition to from 10 c. c. to 18 c. c. silica sol.

5. An investment composition comprising a setting refractory magnesium oxide-water soluble acid phosphate investment material bonded with a silica sol in the ratio of 100 gms. investment composition to from 10 c. c. to 18 c. c. silica sol of 2-30% concentration to give a workable slurry.

6. In the process of making a casting by the lost-wax method from metals melting at over 2300° F., the steps which include producing a cast

of the desired article in a model investment consisting essentially of by weight from 72.5% to 85% of a refractory material, from 17.5% to 10% of a water soluble acid phosphate salt, and from 10% to 5% of fused magnesium oxide, in which 5% to 25% by weight of the refractory material is zirconium silicate, coating said cast with wax, and applying an outer investment to said waxed up model investment, said outer investment consisting essentially of by weight 89% to 71.8% of a refractory material, from 7 to 18.2% of a water-soluble acid phosphate salt, and from 4 to 10% of magnesium oxide, said outer investment being substantially free from zirconium silicate and differing in composition from the model investment and having a lower compression strength than the model investment, a thermal expansion not greater than that of the model investment, and a setting expansion of not more than .2%.

5 10 15

References Cited in the file of this patent  
UNITED STATES PATENTS

| Number    | Name         | Date           |
|-----------|--------------|----------------|
| 1,901,054 | Dailey       | Mar. 14, 1933  |
| 2,057,289 | Birdlebough  | Oct. 13, 1936  |
| 2,072,212 | Moosdorf     | Mar. 2, 1937   |
| 2,195,452 | Erdle        | Apr. 2, 1940   |
| 2,247,586 | Neiman       | July 1, 1941   |
| 2,333,430 | Lee          | Nov. 2, 1943   |
| 2,368,719 | Miller       | Feb. 6, 1945   |
| 2,372,236 | Wainer       | Mar. 27, 1945  |
| 2,380,945 | Collins      | Aug. 7, 1945   |
| 2,394,394 | Miller       | Feb. 5, 1946   |
| 2,461,416 | Erdle        | Feb. 8, 1949   |
| 2,466,138 | Wainer       | Apr. 5, 1949   |
| 2,479,504 | Moore et al. | Aug. 16, 1949  |
| 2,494,403 | Nies et al.  | Jan. 10, 1950  |
| 2,522,548 | Streicher    | Sept. 19, 1950 |